

## UNITED STATES PATENT OFFICE

VICTOR R. ABRAMS, OF BRUNSWICK, GEORGIA, ASSIGNOR TO ARTHUR H. BALLARD, OF BRUNSWICK, GEORGIA

## SULPHUR LUBRICANT

No Drawing. Original application filed April 5, 1932, Serial No. 603,445. Divided and this application filed September 16, 1932. Serial No. 633,541.

My invention aims to provide an improved lubricant, whereby a stable admixture of free sulphur in a water vehicle is made available for lubricating purposes. This 5 application is a division of my co-pending application, Serial No. 603,445, filed April 5, 1932, the latter being a continuation in part of my co-pending application, Serial No. 594,741, filed February 23, 1932.

10 My lubricant is of especial value in the art of cutting and machining metals.

Experiments and tests have shown that 15 free sulphur will serve as a superior cutting lubricant, owing to the fact that at the temperatures involved the sulphur is present between the frictional surfaces as a highly viscous liquid. Sulphur melts at a temperature of 235° F., forming at this temperature a thin, straw-colored liquid. As its 20 temperature is raised, the liquid turns darker and becomes more viscous until at about 370° F. it is so viscous that it can hardly be poured. As the temperature is still further raised, the viscosity decreases, but even 25 at a temperature just below its boiling point (832° F.) it is still much more viscous than is cutting oil at even 240° F.

In addition to this property, which greatly 30 assists in maintaining a proper lubricating film between the frictional surface, other properties are possessed by free sulphur which renders it superior to oil or similarly acting lubricants, for metal cutting and other high temperature purposes.

35 The molten sulphur present at and near the pressure zone not only conducts away heat but the sulphur as it is melted takes up an amount of heat equal to its latent heat of fusion, thus increasing the cooling 40 action.

Furthermore, at the temperatures involved, the sulphur undoubtedly combined with the metal so as to form a sulphide contaminating film, or films, between the 45 faces being lubricated, thereby decreasing

the intersurface molecular adhesion and otherwise reducing the friction between chip and tool.

I am aware that there are a number of so-called "sulphurized" liquids now being 50 used as cutting fluids. These contain in solution sulphur compounds, or contain elemental sulphur in true solution, and in some cases may also contain small amounts of sulphur particles of colloidal size. I have 55 discovered that finely divided free sulphur (by which I mean sulphur particles of greater than colloidal size) will itself function as a cutting lubricant which is far superior to any of the cutting lubricants containing sulphur in other forms heretofore used, and that this finely divided free sulphur possesses lubricating qualities different from, and in addition to, the qualities possessed by sulphur in other forms. This 60 great superiority becomes the more marked at exceptionally high cutting speeds and when difficultly machinable metals are cut.

From a practical standpoint, the sulphur is advantageously in a liquid vehicle, so that 70 it may be readily introduced into the zone of action. If finely divided sulphur (flowers of sulphur) is stirred with oil, water or other liquid vehicles, it will not stay in suspension but will settle out and hence would 75 have to be stirred until almost the time for application in order to be utilized. This is highly inconvenient and therefore impractical as a general proposition.

80 In accordance with my invention, I am able to prepare stable, mobile, admixtures of finely divided sulphur and liquid vehicles, which may contain as much or more than 40% of free sulphur. The great bulk 85 of these sulphur particles, as my product is normally prepared, are greatly above colloidal size, and in practice may be of sufficient size as to be easily visible to the naked eye. The liquid vehicle serves principally 90

as a carrier for the sulphur so that it may be introduced to the zone of lubrication, and does not itself function, except perhaps to a slight incidental degree, as a lubricant.

5 I may employ water as a vehicle. In order to maintain the sulphur particles, which in practice will be mainly non-colloidal in size, in a stable suspension, I employ various "stabilizers", which have the 10 property of actually sustaining the sulphur particles, or causing them to be sustained, in the liquid vehicle or carrier for long periods of time. Although these stabilizing substances do increase the viscosity of the 15 vehicle somewhat, this is purely incidental. The effect with which I am concerned is not that of merely delaying the settling out of the sulphur particles but that of causing them to be sustained for indefinitely long 20 periods of time so as to obtain stable suspensions of free sulphur. By "stable" I do not mean necessarily absolute stability but stability in the sense that there is little or no separation or settling out of the sulphur particles.

When using a water vehicle, I employ such substances for "stabilizers" as starch, gums, glue, casein, dextrin, and the like. 25 These "stabilizers" which I employ may be broadly characterized as being gel-forming materials.

Irrespective of what may be the correct explanation for the stabilizing action, I have 30 found in the course of my work that my sulphur mixtures behave as though comprising a discontinuous gelatinous mass composed of particles of elastic gel in contact with each other and having the interspaces containing a liquid, the sulphur particles being 35 distributed between the gel particles and supported thereby. The mass may properly be termed a "fluid gel", or a "freely flowing gel", because it acts like liquid which will 40 flow freely and may be readily poured, although largely composed of gel. Upon standing, such mixtures often exude a serum 45 comprised of the liquid contained between the gel particles, forming a layer distinct 50 from the gelatinous mass, the sulphur remaining distributed throughout the latter and stably suspended therein. Gentle agitation 55 or stirring readily causes the serum layer to redistribute itself throughout the gel to reform the original mixture.

Having discussed the properties and nature of my stable sulphur suspensions, and the theory so far as it is known to me, so 60 that others skilled in the art may be better able to proceed in amplifying the list of sulphur stabilizers which I have specifically named, and in properly using them, I will 65 now describe in detail an illustrative embodiment of my invention.

### Example

1% to 5% of starch is mixed with water and the whole heated, as by blowing in steam, to the boiling point. The resulting 70 mixture can be thickened or thinned as desired. Allow to cool, preferably without agitation, and add from 5% to 25%, by weight, of powdered sulphur. A germicide, or fungicide, such as carbolic acid, may be 75 added to inhibit coagulation of the starch, although the sulphur present may exert a sufficient germicidal effect.

In a modification of this example, glue, 80 dextrin, casein (with alkali) and similar substances may be used in place of starch or mixed with it.

A fatty or mineral oil may be added to prevent the lubricant from rusting the iron or steel which is exposed to it, and from 85 1% to 15% of ordinary soap may be added to increase the wetting of the surface to be lubricated.

Practical tests have demonstrated that 90 extremely satisfactory results can be secured with my lubricant when operating at high rates of cut. The wear on the tool is much less, the tool maintains its edge for a longer period, and a smoother cut is produced. Tests have shown that tools which would 95 not function with cutting media heretofore employed in the art can be satisfactorily used. Friction and heat are reduced and the operation may be speeded up.

Two instances are given which typify the 100 superior results obtained with my lubricant:

### Drilling Monel metal

1/8" holes drilled in 1/16" metal. With no lubrication, drill destroyed after 1 1/2 holes. 105 With regular petroleum lubrication, drill destroyed after 10 holes drilled. With sulphur lubricant in water vehicle (starch stabilizer), the drill was merely dulled after 110 50 holes.

### Cutting bolts by machine

Old machine used and with lard oil (considered one of the finest cutting lubricants) 115 2 to 3 operations required to produce a good thread on 3/4" bolts. Using my sulphur lubricant, the machine was speeded up to maximum speed and only one operation required to give a good thread. One bolt produced per minute as against one per five 120 minutes with lard oil lubrication.

It can also be used as a lubricant for bearings and frictional surfaces generally and is especially advantageous when the temperatures are abnormally high. Thus it 125 is very satisfactory for use on hot boxes and on heavy bearings where high temperatures are likely to develop, such as bearings on railway cars, journals, etc.

By a "freely flowing lubricant" is meant 130

a lubricant which will flow freely at normal temperatures through circulating pipes that are used in the machine tool art for applying cutting fluids to the cutting point, 5 and which is not viscous enough to support sulphur in stable suspensions by virtue of the apparent bulk viscosity—in other words, one which is not a paste or a cake.

Attention is called to my co-pending application Serial No. 644,503, filed November 26, 1932.

The invention is obviously not restricted to the embodiments described, but what is claimed is as follows:

15 1. A cutting lubricant gel freely flowing at ordinary temperatures comprising a water vehicle gelled with a small amount of a gel-forming substance selected from the class typified by starch, gum, dextrin, glue and 20 casein; and containing powdered sulphur of greater than colloidal size distributed therethrough in amount to function as a lubricating ingredient and be stably suspended therein.

25 2. A cutting lubricant gel freely flowing at ordinary temperatures comprising a water vehicle gelled with a small amount of starch and having powdered sulphur of greater than colloidal size distributed therethrough in amount to function as a lubricating ingredient and be stably suspended therein.

30 3. A cutting lubricant gel freely flowing at ordinary temperatures comprising a water vehicle gelled with a small amount of gum and having powdered sulphur of greater than colloidal size distributed therethrough in amount to function as a lubricating ingredient and be stably suspended therein.

35 4. A cutting lubricant gel freely flowing at ordinary temperatures comprising a water vehicle gelled with a small amount of casein and having powdered sulphur in greater than colloidal size distributed therethrough in amount to function as a lubricating ingredient and be stably suspended therein.

40 5. A cutting lubricant gel freely flowing at ordinary temperatures comprising a water vehicle gelled with about 1%-5% of starch and having about 5%-25% of powdered sulphur of greater than colloidal size distributed therethrough and stably suspended therein.

45 6. A cutting lubricant freely flowing at ordinary temperatures consisting of a water vehicle and a gel formed of water and a substance selected from the class typified by starch, gum, dextrin, glue and casein distributed therethrough and carrying in stable suspension dispersed free sulphur particles of greater than colloidal size in sufficient amount to function as the lubricating ingredient, thereby permitting exceptionally

high speed cutting, and said gel serving to minimize the corrosive action of the sulphur when the latter is not actually being employed to produce lubrication of the cutting tool where it engages the work.

7. The method of preparing a freely flowing cutting lubricant gel containing powdered sulphur of greater than colloidal size stably suspended in a water vehicle, comprising mixing and heating together until 75 solution is effected a water vehicle and a small amount of a gel-forming substance selected from the class typified by starch, gum, dextrin, glue and casein, cooling said mixture and allowing a gel to form, and distributing powdered sulphur of greater than colloidal size 80 throughout the gel by mixing therewith, said mixing rendering the gel freely flowing and said gel-forming substance being in sufficient amount to cause 85 said sulphur to be stably suspended.

8. The method of preparing a freely flowing cutting lubricant gel containing powdered sulphur of greater than colloidal size stably suspended in a water vehicle, comprising 90 mixing and heating together until solution is effected a water vehicle and a small amount of gum, cooling said mixture and allowing a gel to form, and distributing powdered sulphur of greater than colloidal size 95 throughout the gel by mixing therewith, said mixing rendering the gel freely flowing and said gel-forming substance being in sufficient amount to cause said sulphur to be 100 stably suspended.

9. The method of preparing a freely flowing cutting lubricant gel containing powdered sulphur of greater than colloidal size stably suspended in a water vehicle, comprising mixing and heating together until 105 solution is effected a water vehicle and a small amount of casein, cooling said mixture and allowing a gel to form, and distributing powdered sulphur of greater than colloidal size throughout the gel by mixing therewith, 110 said mixing rendering the gel freely flowing and said gel-forming substance being in sufficient amount to cause said sulphur to be 115 stably suspended.

10. The method of preparing a freely 115 flowing cutting lubricant gel containing powdered sulphur of greater than colloidal size stably suspended in a water vehicle, comprising mixing and heating together until solution is effected a water vehicle and a 120 small amount of starch, cooling said mixture and allowing a gel to form, and distributing powdered sulphur of greater than colloidal size throughout the gel by mixing therewith, said mixing rendering the gel freely 125 flowing and said gel-forming substance being in sufficient amount to cause said sulphur to be stably suspended.

11. The method of preparing a freely flowing cutting lubricant gel containing 130

powdered sulphur of greater than colloidal size stably suspended in a water vehicle, comprising mixing together water and about 1%-5% of starch, agitating the mixture at 5 about its boiling point until solution is effected, cooling and allowing a gel to form, and distributing about 5%-25% of powdered sulphur of greater than colloidal size throughout the gel by mixing therewith.

10 In testimony whereof, I have signed my name to this specification.

VICTOR R. ABRAMS.

15

20

25

30

35

40

45

50

55

60